# EUROPEAN PATENT APPLICATION

(11) **EP 0 903 163 A1**
(43) Date of publication of application: **24.03.1999**
(21) Application number: 97925336.6
(22) Date of filing: 24.04.1997
(51) Int. Cl.: A62C 3/00, A62C 5/00, A62D 1/00

(54) **MINERAL-WATER SUSPENSION FOR USE AGAINST FIRES**

(30) Priority: 24.05.1996 RU 96110494
(71) Applicant: Mezhdunarodny Fond Popechitelei Moskovskogo Gosudarstvennogo Aviationnogo Tekhnologicheskogo Universit Imeni K.E.Tsiolkovskogo, Moscow, 103767 (RU)
(72) Inventor: GUROV, Alexandr Ivanovich, Moscow, 113076 (RU); ODNOVOL, Leonid Alexandrovich, Moscow, 127322 (RU); SYTNIKOV, Alexandr Nikolaevich, Moscow, 123481 (RU)
(74) Representative: Kidd, Piers Burgess
(86) International application number: RU9700127
(87) International publication number: WO9745166

(57) **Abstract**

The proposed fire-fighting mineral-water suspension can be used for extinguishing and preventing fires of different kinds and intensity and comprises water glass, clay and water, wherein it comprises water glass with its weight ratio to clay being from (1:1) to (1:10), respectively.

## Description

### Field of the Invention

The present invention relates to materials for extinguishing and preventing fires, and more concretely - to a fire-fighting mineral-water suspension.

### Background Art

Systems of state and public measures are widely known, which are carried out in order to prevent fires, to limit the spread of fires which have started, and to successfully extinguish different kinds of fires of different intensity. A composite part of such systems is the development of new agents, including different materials, comprising ecologically clean components of natural origin and being highly effective at low cost.

Water is widely known as a fire-extinguishing agent. However, water can only be used to extinguish fires, not to prevent them. Wherewith, the low efficiency of that agent results in a large consumption thereof For example, when forest fires are to be extinguished, about 12-15 kg/m² of water is necessary, but this amount cannot always be provided in the situation at hand.

Various solutions of retardants (agents slowing up the spread or intensity of a fire) in water are also widely known. However, as a rule, retardants are complex chemical compounds (for example, on the base of diammonium phosphate) which contaminate the environment and also require the use of a complex manufacturing process, complex equipment for mixing and delivering to the location of the fire (reservoirs and drain devices of a complex construction, controlling the manufacturing process with a computer). All of this results in a substantial increase in the cost of extinguishing a fire and substantially reduces the possibility of using them for the purpose of prevention.

Fire-fighting water suspensions comprising components of natural origin, for example, sand, clay and water, are also known (SU, A, 494164, A6 201/10, 1973; SU, A, 626780, A6 201/10, 1976).

Wherein, the known water suspension (SU, A, 626780) comprises the aforesaid components in the following relationship, % by weight.

| | |
|---|---|
| sand | 5-20, |
| clay | 1-5, |
| water | balance. |

The aforesaid compositions are ecologically clean and cheap products. However they have rather low adhesive and insulating properties which do not make it possible to hold the moisture on the surface being treated until there is complete evaporation of the water or to reliably insulate the product of pyrolysis. This is explained by the fact that sand is a loose rock, consisting mainly of grains of different minerals and fragments of ore of a size of from 100 to 5000 microns, and has an insignificant admixture of aleurite and clay particles (the latter not more than 3%) of a size of from 10 to 100 microns. The presence of the aforesaid large fractions, insoluble in water, results in the formation of a sediment in the suspension, which is also abrasive material in respect of fire-fighting equipment (pipelines, discharge devices and the like). Furthermore, even though the presence of clay enhances the adhesive properties of the composition, the presence of the sand in practice neutralizes these properties, since sand has a high looseness and this does not make it possible to hold the components of the suspension (in particular, the water) on the surfaces being treated.

All of the foregoing limits the use of the aforesaid suspensions and makes it possible to use them, mainly, to extinguish and localize steppe fires.

### Disclosure of the Invention

At the base of the present invention lies the object of creating a fire-fighting mineral-water suspension with such components which would ensure enhancement of its adhesive and insulating properties, this making it possible to use the suspension to both extinguish and to prevent fires.

This object is achieved by creating a fire-fighting mineral-water suspension comprising clay and water, which in accordance with the invention additionally comprises water glass in a weight ratio to clay of from (1:1) to (1:10), respectively.

The presence of water glass substantially enhances the adhesive and insulating properties of the proposed suspension. This is due to the fact that water glass has high adhesive properties, is easily dissolved in water, does not cause the formation of a sediment, and makes it possible to hold particles of clay in a suspended state. Wherein, the water glass in combination with clay holds the water on the surface being treated until it completely evaporates, irrelative of the angle of inclination of that surface to the horizon Furthermore, after evaporation of the water, a coating of silicon oxides is formed on the treated surface, which prevents the access for oxygen to the heart of the fire, and also prevents the inflow of energy, both from the heart of the fire, which limits its spreading, and to that heart, which eliminates the possibility of repeated combustion

The aforesaid properties of the proposed suspension make it possible to use it in the case of fires of different kinds and intensity, in particular:
- city fires: when extinguishing fires in dwellings and work buildings, and also other administrative, scientific, educational and such structures;
- forest and steppe fires: extinguishing those fires themselves and also protection of adjacent territory against those kinds of fires;
- fires in oilfields, and also fires of spilled petroleum products as a result of accidents and natural calamities.

Wherein, the effectiveness of use of the proposed suspension is tens of times greater than the effectiveness of using, for example, water. That is, the consumption of water during the extinguishing of for example, a forest fire is, on the average, 12-15 kilograms per square meter of the burning surface, while the consumption of the proposed suspension is 0.12-0.15 kilograms per square meter to achieve the same result, which substantially reduces expenditures on extinguishing fires, especially intensive and large-scale fires.

Furthermore, the aforesaid qualities of the proposed suspension make it possible to substantially expand the field of its use. That is, it can not only be used to extinguish fires, but also to prevent them, for example, to cover surfaces of combustible materials inside buildings and structures, and also to cool and insulate surfaces neighboring with the heart of a fire.

In order to extinguish different kinds of fires, it is advisable to use a suspension comprising water glass with its weight ratio to clay being from (1:1) to (1:10), respectively, and the total content of water glass and clay in the suspension is from 60 to 80 % by weight, the balance water.

Wherein, it is possible that the suspension would comprise components with the following ratio therebetween, % by weight:

| | |
|---|---|
| water glass | 7-16, |
| clay | 13-72, |
| water | balance. |

The proposed fire-fighting mineral-water suspension has high adhesive and insulating properties, which makes it possible to use it both for extinguishing fires of different kinds and intensity, and for preventing fires.

### Best Method for Carrying Out the Invention

The proposed fire-fighting mineral-water suspension comprises water glass, clay and water. Wherein, the suspension comprises water glass in an amount ensuring its weight ratio to clay from (1:1) to (1:10), respectively. That is, in the suspension there are from 1 to 10 weight parts of clay per one weight part of water glass. Wherein, in order to extinguish fires, it is better to use a suspension in which there is from 1 to 6 weight parts of clay per one part of water glass (a weight ratio from [1:1] to [1:6], respectively), while to prevent fires it is better to use a suspension in which there is from 4 to 10 weight parts of clay per one part of water glass (weight ratio from [1:1] to [1:10], respectively).

The sum content of water glass and clay in the suspension may vary from 20 to 80 % by weight, the balance water. Wherein, the following content of the components in the suspension is possible, % by weight:

| | |
|---|---|
| water glass | 7-17, |
| clay | 13-72, |
| water | balance. |

An aqueous solution of, for example, sodium silicate or potassium silicate may be used as the water glass.

With the aforesaid ratios of the water glass, clay and water, each particle of the clay is coated with a solution of water glass and is held in the suspension in a suspended state.

This ensures homogeneity of the suspension, facilitates its breakup into drops during spraying, since the water glass reduces the surface tension of the suspension.

If the weight amount of water glass in the suspension relative to the weight amount of clay is less than 1:1, then the amount of water glass will be insufficient to hold all the particles of clay in a suspended state, which will result in a reduction of the insulating properties of the suspension.

If the weight amount of clay in the suspension relative to the weight amount of liquid glass will be greater than 10:1, then it will be difficult to apply the suspension onto the surface being treated, and it will also be difficult to hold the suspension on that surface, since due to the large amount of clay, the friability of the suspension will substantially increase when the water evaporates.

If the content of water glass in the suspension is reduced to less than 7 % by weight, then the effect of holding the particles of clay in a suspended state may be impaired. Furthermore, the aforesaid reduction of the content of water glass may result in a reduction of the insulating properties of the suspension, since the water glass may be insufficient to form a coating of silicon oxides on the treated surface alter evaporation of the moisture.

If the content of the water glass is increased to more than 16 % by weight, then the density of the suspension increases, which may result in difficulties when it is supplied to the heart of a fire.

If the content of clay in the suspension is reduced to less than 13 % by weight, then the adhesive properties of the suspension are impaired, as a result of which it will be difficult to hold moisture on the surface being treated until complete evaporation of the moisture.

If the content of clay is increased to more than 72 % by weight, then the problem of converting it into a finely dispersed state and obtaining a homogeneous suspension arises, which may cause difficulties when it is supplied to the heart of a fire. Furthermore, the viscosity of the suspension increases thereby.

The proposed suspension is prepared in the following manner.

At first, water glass is dissolved in water, then clay is added to the obtained solution and stirred, for example, in a concrete mixer to a homogeneous state. In order to reduce the time for preparation, it is advisable to preliminarily grind the clay.

The prepared suspension is a microheterogeneous freely-dispersed system in which water is the dispersing medium, and water glass and clay are the dispersed phase. Wherein, the ratio between the latter may vary within the aforesaid wide ranges, which does not substantially affect the fire-extinguishing and fire-retardant properties of the suspension. Wherein, the suspension has high adhesive and insulating properties.

The quantitative make-up of the components in the suspension, as indicated above, is determined by its purpose, i.e. whether it is used as a fire-suppressing or a fire-retardant agent.

Thus, for example, when a fire is being extinguished in dwellings, it is advisable to use a solution with a low sum content of clay and water glass (about 20 % by weight, balance - water), since the main object is to cool the heart of the fire. At the same time, it is advisable that the walls of buildings neighboring with the heart of the fire be covered with a composition having a higher sum content of those components (about 60-80 % by weight, the balance - water). There should be a similar approach when extinguishing fires at enterprises, storehouses, warehouses and other similar structures.

When forest and steppe fires are to be extinguished, the most optimum solution is when the sum content of clay and water glass is 40-60 % by weight, since this make-up, as experiments with models and artificially caused real forest fires showed, has good cooling (water in a finely dispersed state is held on the hot surface) and insulating (a sufficiently large amount of clay and water glass) properties.

The amount of water within the aforesaid limits depends on the purpose of the suspension, and reduction of its content below the lower limit or an increase of its content above the upper limit results in the need to increase or reduce the content of the dispersed phase in the suspension, which may result in the negative consequences described above.

The prepared suspension is used by spraying with different existing methods (for example, by means of pumps, pouring from planes or helicopters). Methods of dispersing, using the energy of an explosion or pressure accumulators (for example, air, powder) are the most effective methods, since they make it possible to disperse a suspension to drops having a diameter of less than 10 microns, substantially increasing thereby the surface of interaction with the flame.

For better understanding of the invention, concrete examples of embodiment thereof are presented below.

### Example.

The proposed suspension was prepared in accordance with the method described above with different amounts of the components therein. Then its fire-retardant properties were determined with wooden samples which were standard matches with removed heads. The wooden samples were covered with the proposed suspension with different amounts of the components therein, put in the flame of a gas burner (the temperature of the burner flame was 1150±20°C), and the time until the sample began to burn or until it began to smolder was determined, since in the majority of cases, a coating of a solid solution of water glass and clay was formed on the sample alter evaporation of the water. Wherein, the temperature inside the coating was not sufficient for combustion of the sample, and only caused its slow smoldering which was determined by the appearance of smoke from under the coating at the end faces of the sample.

For comparison the time of combustion of a sample preliminary treated with water was determined.

Different ratios of the components in a suspension having a volume of approximately 0.04 m³, and also the time prior to their combustion (the beginning of soldering) are presented in the examples, tabulated below, in which for comparison the time prior to combustion of the sample treated with water is presented in example No. 31

**Table**

| No. | Sum content of water glass and clay, % by weight | Ratio of water glass to clay, weight parts (approx) | Content of components % by weight water clay water glass | | | Time prior to combuston (beginning of smoldering) of the sample, seconds |
|---|---|---|---|---|---|---|
| 1 | 2 | 3 | 4 | 5 | 6 | 7 |
| 1 | 20 | 1:1.9 | 7 | 13 | 80 | 7.8 |
| 2 | 26 | 1:1.6 | 10 | 16 | 74 | 7.7 |
| 3 | 21 | 1:3.2 | 6 | 19 | 75 | 10.1 |
| 4 | 25 | 1:5.5 | 4 | 21 | 75 | 11.7 |
| 5 | 25 | 1:7.4 | 3 | 22 | 75 | 11.2 |
| 6 | 47 | 1:1.8 | 17 | 30 | 53 | 9.2 |
| 7 | 47 | 1:3.7 | 10 | 37 | 53 | 12.9 |
| 8 | 47 | 1:4.9 | 8 | 39 | 53 | 14.0 |
| 9 | 47 | 1:6.9 | 6 | 41 | 53 | 12.6 |
| 10 | 67 | 1:1.8 | 24 | 43 | 33 | 11.2 |
| 11 | 67 | 1:3.5 | 15 | 52 | 33 | 17.4 |
| 12 | 67 | 1:5.1 | 11 | 56 | 33 | 18.0 |
| 13 | 67 | 1:6.5 | 9 | 58 | 33 | 15.6 |
| 14 | 85 | 1:1.8 | 31 | 54 | 15 | 14.5 |
| 15 | 84 | 1:3.5 | 19 | 65 | 16 | 25.6 |
| 16 | 85 | 1:5.6 | 13 | 72 | 15 | 23.8 |
| 17 | 84 | 1:7.4 | 10 | 74 | 16 | 18.9 |
| 18 | 25 | 1:7.4 | 3 | 22 | 75 | 8.2 |
| 19 | 25 | 1:1.3 | 11 | 14 | 75 | 7.0 |
| 20 | 26 | 1:1 | 13 | 13 | 74 | 5.5 |
| 21 | 44 | 1:10 | 4 | 40 | 56 | 10.4 |
| 22 | 47 | 1:2.6 | 13 | 34 | 53 | 11.3 |
| 23 | 47 | 1:4.9 | 8 | 39 | 53 | 14.0 |
| 24 | 66 | 1:8.5 | 7 | 59 | 34 | 11.0 |
| 25 | 66 | 1:4.5 | 12 | 54 | 34 | 18.3 |
| 26 | 66 | 1:2.7 | 18 | 48 | 34 | 15.3 |
| 27 | 84 | 1:8.4 | 9 | 75 | 16 | 13.5 |
| 28 | 84 | 1:6 | 12 | 72 | 16 | 21.5 |
| 29 | 80 | 1:4 | 16 | 64 | 20 | 25.6 |
| 30 | 80 | 1:9 | 8 | 72 | 20 | 16.3 |
| 31 | - | - | - | - | 100 | 4.1 |

As is evident from the presented examples, the time prior to combustion of a sample treated with the proposed suspension, with any content therein of the indicated components, is from about 1.5 to more than 6 times greater than the time required for combustion of a sample treated with water.

Furthermore, the formation of a solid coating of water glass and clay on the surface of the samples, preventing combustion of the samples, clearly demonstrates the high adhesive and insulating properties of the proposed suspension.

### Industrial Applicability

The proposed invention may be used as a fire-suppressing or fire-retardant agent in the case of fires of different kinds and intensity, in particular: city fires, forest and steppe fires, fires at oil fields. Furthermore, the proposed suspension may be used for the prevention of fires, and also for the protection of objects neighboring with the heart of the fire against combustion by applying it onto the surface of items of combustible materials inside different structures or on surfaces adjacent the heart of a fire.

## Claims

1. A fire-fighting mineral-water suspension comprising clay and water, characterized in that it additionally comprises water glass with its weight ratio to the clay being from (1:1) to (1:10), respectively.

2. A fire-fighting mineral-water suspension according to claim 1, characterized in that it comprises water glass with its weight ratio to clay being from (1:1) to (1:6), respectively.

3. A fire-fighting mineral-water suspension according to claim 1, characterized in that it comprises water glass with its weight ratio to clay being from (1:4) to (1:10), respectively.

4. A fire-fighting mineral-water suspension according to claim 1, characterized in that it comprises components in the following relationship, % by weight:
| | |
|---|---|
| sum content of water glass and clay | 20-80, |
| water | balance. |

5. A fire-fighting mineral-water suspension according to claim 1, characterized in that it comprises components in the following relationship, % by weight:
| | |
|---|---|
| water glass | 7-16, |
| clay | 13-72, |
| water | balance. |
